

July 30, 1940.

W. LAUTSCH

2,209,821

METHOD OF SENSITIZING FOUNDATION MEMBERS FOR ELECTRIC DISCHARGE DEVICES

Filed April 26, 1938

Fig. 1.



Fig. 2.



Inventor:  
Werner Lautsch,  
by *Harry E. Deinham*  
His Attorney.

## UNITED STATES PATENT OFFICE

2,209,821

METHOD OF SENSITIZING FOUNDATION  
MEMBERS FOR ELECTRIC DISCHARGE  
DEVICESWerner Lautsch, Berlin-Reinickendorf, Germany,  
assignor to General Electric Company, a corpora-  
tion of New YorkApplication April 26, 1938, Serial No. 204,404  
In Germany May 15, 1937

2 Claims. (Cl. 250—27.5)

The present invention relates to an improved process for coating a foundation member, such as a plate of metal, oxidized or otherwise treated, with a homogeneous layer of sensitive material. Plates of this character have various uses in the art depending upon the character of the sensitive material. For example, when the foundation member is coated with caesium oxide, the surface not only responds to light but also   
10 fusely emits secondary electrons when struck by primary electrons traveling at considerable velocities. In order to coat a number of these plates simultaneously with the sensitive material, it has been customary to mount the plates in an enclosed chamber and to condense the sensitive material from a vapor onto the plates. However, it has been found that when the plates are arranged fairly close together, the directions from which the vapor was condensed were such   
15 that the outer edge of the plates became more heavily coated than the inner portions thereof because the vapor did not have easy access to the innermost spaces between the plates. A tube in which the cathode foundation member   
20 is not uniformly coated gives erratic performance, regardless of whether the cathode is employed as a photo-electric or a secondary emission element.

Accordingly, an object of the present invention is to provide an improved method of coating a foundation member with a layer of sensitive material and having uniform thickness. Other objects are to provide a method by which the layer is formed by condensed particles moving   
25 in random directions which intercept all parts of the surface of the foundation member. A still further object is to provide a coating method which is applicable to those cases where a number of foundation members or plates are arranged close to one another with constricted spaces therebetween and are to be coated simultaneously. These objects are carried out in brief by vaporizing the sensitive material in the presence of gas under pressure whereby the vapor   
30 particles are caused to collide with the gas molecules and are given a multitudinous number of directions through the space about the foundation members. The uniform diffusion of the vapor through the gas causes the vapor to condense on the foundation member as a layer of uniform thickness.

The invention will be better understood when reference is made to the following description and the accompanying drawing in which Fig. 1   
55 shows apparatus for carrying out the improved

process, and Fig. 2 is a diagram useful in explaining the invention.

Referring more particularly to Fig. 1, numeral 1 designates a pair of glass bulbs joined together by a glass tubulation 2 of restricted diameter. A tubulation 3 is provided with a stopcock 4 at one end of the left-hand bulb 1, and an exhaust tubulation 5 is provided at the opposite end of the other bulb 1. Across the tubulation 2 there is a hermetically tight glass diaphragm 6 constructed in any suitable manner so as to fracture easily and, as illustrated, takes the form of a disk with a hemispherical portion at the center, facing the left-hand bulb 1. To the left of the diaphragm 6, there is arranged a sharp, pointed piece of metal 7 with the point positioned to fracture the diaphragm when the metal member is moved either by an external magnet or by gravity. The bulbs 1 are contained in an oven 8, the temperature of which can be regulated or controlled for the purposes which will be explained hereinafter.

The foundation members or plates 9 which are to be coated either with light-sensitive material or with material suitable for secondary emission are mounted in any suitable manner in the right-hand bulb 1 and arranged preferably in a parallel, horizontal position. The plates may be introduced through a large opening (not shown) in the right-hand bulb which is thereafter closed by melting the glass and drawing down to the exhaust tubulation 5. The interior of both bulbs 1 is then highly evacuated by a pump (not shown) connected to the tubulations 3 and 5. The tubulation 5 is thereafter sealed off and the stopcock 4 moved to its closed position. In case the sensitive material to be deposited on the plates 9 is caesium, which is light-sensitive as well as a good secondary emitter, the plates are preferably coated with nickel or silver and then oxidized before being placed in position. The caesium is then introduced into the left-hand bulb in any suitable manner, for example, by heating a capsule (not shown) in the bulb and containing a compound of caesium and a reducing agent, or by distilling the material as a vapor through the tubulation 3. The caesium is indicated by the reference character 10. The oven 8 is then heated to a temperature sufficient to vaporize the caesium but the latter is prevented from reaching the plates 9 by the closed diaphragm 6. The diaphragm may be fractured by moving the weight 7 against the same, which can be conveniently done by means of a magnet on the outside of the tube or by moving the en- 55

tire apparatus to a vertical position and allowing the weight to fall by gravity. The caesium vapor will then enter into the second chamber which is also maintained at an elevated temperature by the oven 8. When the oven 8 is cooled, the caesium vapor condenses on all of the surfaces within the right-hand bulb including the foundation members 9. However, it is apparent that the directions taken by the caesium particles during the condensation step would be such that very little if any of the vapor would condense at the innermost spaces between the plates 9, particularly if the latter were arranged close to one another. The vapor would condense as a heavy layer around the outer edge of the plates, also on the upper surface of the uppermost plate and the lower surface of the lowermost plate. The plates would therefore not have a homogeneous layer of sensitive material over their entire surface and when placed in a photo-electric tube or employed as secondary emitters, would not respond with equal effect to the impinging light rays or electrons over their entire surface.

In accordance with the present invention and as an improvement over the process described up to this point, an inert gas, preferably helium, is employed within the bulb to produce an equal distribution of the vapor throughout the bulb including the spaces between the plates 9. While the pressure of the gas employed for this purpose can best be determined by experiment, depending upon the nature of the gas and of the sensitive material, I find that a pressure of several millimeters in the case of helium is desirable when caesium is being deposited. The pressure of the gas should preferably be such that the mean free path between molecules is less than any dimension of the right-hand bulb 1 so that the vapor particles in moving about the bulb during the condensation process will strike one or more gas molecules, and these elastic collisions will serve to diffuse the vapor uniformly throughout the bulb. Consequently, when the vapor is being condensed on the plates 9, the particles thereof move in countless directions, and these directions necessarily are such as to cause the particles to move freely through the constricted spaces between the plates 9 and to strike all parts of the surface of each plate. The vapor therefore condenses as a uniform layer over the entire surface of each plate and does not tend to condense more rapidly at the outer edges of any one plate or on any other restricted portion thereof.

The manner in which the gas under pressure serves to cause an even distribution of the vapor throughout any and all of the spaces contained within the bulb is clearly shown in the diagram of Fig. 2. The foundation members to be coated are indicated at 9, and the molecules of gas are typified by the small circles 10. It will be noted that these circles are spaced apart considerably less than the diameter of the bulb or combined length of both bulbs to indicate that the mean free path of the gas molecules is less than the important dimensions of the bulb or bulbs. The dotted lines 11 represent the directions taken by

the vapor particles moving through the tube during condensation and colliding with the gas molecules or with the envelope. Inasmuch as these collisions are of an elastic character, the particles enter the constricted space between the plates 9 with great facility and at many different angles and directions, causing the vapor to condense at these inner spaces quite as readily as at the outer spaces near the periphery of the plates.

When the rate of condensation determined by the reduction in temperature of the oven 8 is so rapid as to exhaust the limited supply of caesium vapor before the surfaces are entirely coated, it may be desirable to provide a continually moving stream of vapor in the bulb. The vapor can be introduced through the tubulation 3, either separately or combined with the inert gas. It has been found that when the vapor of a sensitive material is condensed in the presence of gas under pressure, the deposited layer, even though evenly distributed over the entire surface, is of a rough character. This condition is advantageous from the standpoint of multiple reflection of light which strikes the surface when the member is used in a photo-electric tube because the light tends to be reflected several times across each depression formed in the light-sensitive surface. At each reflection or impingement of the light ray on the surface, the light causes increased reaction at the surface which results in an increased light-sensitive effect.

While I have described the invention more particularly in connection with foundation members of a plate form coated with light-sensitive material, it will be understood that the invention is not limited to these features but can be applied to foundation members of any shape or material and to any coating material which can be readily vaporized.

What I claim as new and desire to secure by Letters Patent of the United States, is:

1. In the art of simultaneously sensitizing a plurality of foundation members, the steps of oxidizing said members, then introducing them into an enclosure, heating said members, passing helium at a pressure of several millimeters admixed with caesium vapor through spaces about and between said members, then cooling said members to cause the vapor to condense from random directions onto the entire surface of said members.

2. In the art of simultaneously coating a plurality of foundation members with a sensitizing material, the steps which include assembling the members in juxtaposition, providing relatively constricted spaces between them, supplying vaporized sensitizing material in the vicinity of the assembled members and in admixture with an inert gas at a pressure of the order of several millimeters so as materially to shorten the mean free path of the vapor molecules, thereby to assure their effective penetration into the said constricted spaces, and cooling the foundation members sufficiently to cause the vaporized material to condense thereon.

WERNER LAUTSCH.